

March 12, 1940.

M. STEINSCHNEIDER ET AL

2,193,301

BLEACHING CELLULOSE

Filed July 19, 1938



Inventors:

Max Steinschneider,  
Erich Knopf,  
By Potter, Pierce & Schaffler,  
Attorneys.

## UNITED STATES PATENT OFFICE

2,193,301

## BLEACHING CELLULOSE

Max Steinschneider and Erich Knopf, Berlin,  
Germany, assignors to Aschaffenburger Zell-  
stoffwerke Aktiengesellschaft, Berlin, Germany

Application July 19, 1938, Serial No. 220,116  
In Germany July 22, 1937

3 Claims. (Cl. 8—105)

This invention relates to a method of bleaching cellulosic fibers with chlorine and more particularly with chlorine gas.

Quite a number of methods of bleaching cellulosic fibers are already known, in which use is made of chlorine, and especially chlorine gas or other substances containing or yielding chlorine.

The defect of known methods consists essentially in that it is not possible to dose the chlorine so accurately, in respect of its time of action on the fibers, and to bring it so intimately into contact with the fibers, at the moment of the reaction, as to prevent the cellulose itself from being also attacked. Losses of and injuries to the cellulose consequently result.

It has now unexpectedly been ascertained in accordance with the present invention that these disadvantages can be reliably avoided by forcing a slurry of the cellulosic fibers to be bleached under pressure through a jet apparatus, for example by means of a pump, and drawing in chlorine gas, supplied in any desired manner, by the reduced pressure thus produced in the jet apparatus. In consequence of the resulting flowing and whirling, very thorough mixing of the slurry and chlorine gas takes place, in such a way that the chlorine is absorbed extremely quickly and completely by the fibers, in fact so quickly that the chlorine has no time to have an oxidizing action on the cellulose itself, but only chlorinates the lignin, the latter being converted into a form in which it is readily soluble in water or dilute alkali and can easily be removed from the cellulose by simple washing out, while the cellulose itself remains entirely unaffected. The result attained by the present invention is evidenced by the constant molecular weight of the cellulose before and after bleaching.

The action of the chlorine on the fibers can be regulated in various ways for example by varying the concentration of the stuff mixture, or by varying the speed of the pump feeding the jet apparatus.

The following is an example of the manner in which the process is carried out.

The fibers to be bleached, e. g., wood pulp, are forced in suspension in a carrier liquid, e. g., water, by a pump through a jet apparatus, its concentration being from 1 to 3%, and the

amount of chlorine gas required for the chlorination is drawn into the jet apparatus under the action of the resulting reduced pressure. After a relatively short time of reaction between the fibers and the chlorine, the chlorinated lignin is removed by washing with water or dilute alkali.

In order more clearly to understand the invention, reference is made to the accompanying drawing, which illustrates diagrammatically and by way of example one embodiment of apparatus suitable for carrying the invention into practical effect, and in which—

The fibers to be treated pass in the form of a suspension, from the container 1 into the suction line 2 of a centrifugal pump 4 driven, for example, by the electric motor 3, which pump forces the suspension through the pipe 5 into and through a jet apparatus 6 of known construction. A supply line 8 is connected at 7 to the jet apparatus for the chlorine gas which is drawn by suction 20 into the jet apparatus. The latter, strictly speaking its diffusor, is contained by a pipe line 9. The action of the chlorine gas drawn in by the jet apparatus on the fibers starts in the diffusor and in this pipe line 9. However a special reaction chamber (not shown) may be connected to the line 9.

The suspension may be forced into and through the jet apparatus by a different device or arrangement, instead of a pump. In addition, chlorine-containing liquids or other substances containing or yielding chlorine may be drawn in with the aid of the jet apparatus, instead of chlorine gas.

We claim:

1. In the method of bleaching cellulose pulp suspension with chlorinating agent the steps comprising, forcing the pulp through a jet apparatus, drawing the chlorinating agent into the jet apparatus solely by the suction resulting therein, whereby intimate contact and mixture takes place in the diffusor of said jet apparatus between the chlorinating agent and the pulp.

2. Method as defined in claim 1 in which the chlorinating agent comprises gaseous chlorine.

3. Method as defined in claim 1 in which the chlorinating agent consists of gaseous chlorine.

MAX STEINSCHNEIDER.  
ERICH KNOFF.